

# UNITED STATES PATENT OFFICE.

WILLY WOLFF, OF MILWAUKEE, WISCONSIN, ASSIGNOR TO RADIUM CHEMICAL COMPANY, OF MILWAUKEE, WISCONSIN, A CORPORATION OF WISCONSIN.

## DEVELOPER FOR DYED FABRICS.

1,311,150.

Specification of Letters Patent.

Patented July 22, 1919.

No Drawing.

Application filed February 1, 1917. Serial No. 145,830.

To all whom it may concern:

Be it known that I, WILLY WOLFF, a subject of the Emperor of Germany, residing at Milwaukee, in the county of Milwaukee 5 and State of Wisconsin, United States of America, have invented a certain new and useful Improvement in Developers for Dyed Fabrics, of which the following is a full, clear, concise, and exact description.

10 My invention relates to the art of dyeing fabrics and is concerned with certain processes of dyeing and with certain dyestuffs employed in such processes.

15 My invention is based fundamentally upon the preliminary use of dyes which are of themselves incapable of giving fast color to fabrics or of giving a particular desirable gloss of finish, and particularly are incapable of giving a satisfactory black. I mention black particularly because of the standard created, for instance, by the so-called "Sambesi black" well known in the art as resulting in consequence of the oxidization 20 of a preliminary treatment by a so-called "developer" after the preliminary treatment had been prepared for such oxidation by an acid bath, the final color being due largely to the oxidization which has been referred to. The result is a fast blue black and the 25 fabric thus dyed has a satisfactory finish. This process is limited absolutely to the production of black, and possibly brown materials.

30 My invention looks toward all dyestuffs, and particularly so-called "direct" dyes which, as employed heretofore, resulted in unstable colors without any particularly desirable gloss or finish to the fabric. It is important that, in the case of these direct 35 dyes, various colors may be obtained and therefore, when I am able to get a satisfactory black or brown with a direct dye, I am not only equaling the possibilities of the Sambesi black and brown, but I go beyond

the possibility of such a process described 45 above in that the black which I secure is a deep green black, preferable to the Sambesi blue black, in that I am able to secure other colors of fast quality, in that I obtain a better luster than that resulting from the Sambesi process, and in that the fabric is less deleteriously affected than in the Sambesi process.

45 I am aware that certain dyes of the amido group have been developed after a fashion, 55 but my invention is not limited in its application to the amido group alone but is applicable to practically any dye and even in the case of the amido dyes gives a better color, a permanent color, and that with less total 60 dyestuffs than heretofore employed. Therefore, as far as the amido group is concerned I provide an improved process and an improved "developer" and my invention goes beyond that in that it is applicable beyond 65 the amido group. In the prior art where developing is done a large displacement of elements takes place with a consequent considerable loss, while according to my invention the developer completes the action with- 70 out entailing such losses, cutting down the required total dyestuffs necessary for a given consignment of fabric from five to fifty per cent.

75 Referring first to the matter of securing a black by my process, I shall speak particularly of "direct" dyes and I shall point out first that it is well known in the art that in dyeing fabrics with what those skilled in the art know as a "direct" black, a brownish 80 black resulted, unstable and without any particularly desirable gloss or finish, as above pointed out. A finishing process, known to the art, is employed, this finishing process following the ordinary dyeing by 85 immersion and consisting of a formaldehyde treatment which tends to set the color, but which does not do so absolutely or even satis-

factorily and which gives no gloss or desirable finish.

According to my invention I "develop" any dye and particularly so-called direct dyes. I use the word "develop" since what I do is to treat an unfinished fabric, dyed by direct dye, for instance, to change the brownish black to a fast deep green black with a high luster and desirable finish. In 10 other words, I first employ the ordinary dyeing by immersion and then after preparation, I treat the fabric according to the processes to which I shall presently refer in detail. I treat, for instance, a direct dye 15 unfinished fabric to get a deep green black, preferable to a blue black, to set the color permanently, and to finish with a high luster.

I have determined the reagents, which I 20 use, by experiment. I have successfully used the processes described herein with the results set forth and in order fully to advise those skilled in the art I shall state precisely the reagents which I employed, the proportions which I actually used, and the other 25 conditions under which I have done the work, it being understood that departure may be made without parting from the spirit and scope of my invention, and that the 30 scope of my invention is to be determined by the appended claims which are carefully drawn of various scope in order to protect the broad as well as specific features of my invention. For illustration, I shall describe 35 my invention as proceeding with a direct dyed fabric.

A direct dyed fabric may be produced by 40 treating the fabric in the usual way with a direct black dye, such for instance, as diamon black or diamine black, BO, such as described on pages 89 and 111, respectively, of the "Chemistry of Dyestuffs" by George Von Georgievics, published by Scott, Greenwood & Co., London, (1903).

45 Since the immersion and dyeing by these direct dyes is well known that process need not be set forth here. The fabric, dyed as just pointed out, is then treated in an acid bath in preparation for the succeeding steps.

50 This acid bath is as follows:

$\frac{1}{2}$  pound sodium nitrite (crystal form).  
 $\frac{1}{2}$  pound sulfurous acid or sulfuric acid.  
100 gallons water.

55 This is an example of a so-called diazotizing bath. The bath is conveniently used at room temperature and a bath according to the above formula is sufficient for a hundred pounds of fabric. It is sufficient to 60 allow the fabric to remain in the bath about fifteen minutes.

The superfluous materials are then washed out of the fabric by means of cool or cold water and the fabric is then subjected to the "developing" bath. This should be done 65 promptly since light affects the fabric in this condition. To describe this developing bath I shall first give the ingredients as follows:

- (1) 80 gr. acetic acid 30%.  
(2) 80 gr. chloroform.  
(3) 80 gr. zinc acetate.  
(4) 10 gr. aqua ammonia 26%.  
(5) 880 gr. cold water.  
(6) 5 lb. beta naphthol.  
(7) 1 lb. alpha naphthylamin.  
(8) 3 lb. phenol (crystallized).  
(9) 8 lb. caustic soda.

These materials are added together and 80 are heated to complete fusion. To this 75 $\frac{1}{2}$  pounds sodium chlorid is slowly added and thoroughly mixed. Then 5 pounds nitric acid or hydrochloric acid is slowly and carefully added. The whole is then cooled off 85 and then pulverized, resulting in 100 pounds developing material. Four to eight ounces of this developing material is diluted in sufficient boiling water to form a solution and this solution is added to sufficient cold 90 water to overflow the hundred pounds of fabric heretofore mentioned.

The acid prepared fabric is allowed to remain in this developing bath for about fifteen minutes during which the color 95 changes to a deep green black, the color is permanently set and the high luster finish is given. Thereupon the fabric is removed from the bath and is washed out in warm or hot water and soap to take out the superfluous developer and any other loose foreign matter, this step also testing the fabric for permanency of color.

I have tried my treatment described herein on colors other than the direct black 105 above set forth and with success and it will therefore be clear that my invention may be employed advantageously in the treatment of any direct dyed fabric. I have also tried my treatment on dyes other than "direct" 110 dyes and on dyes other than of the amido group, with successful results. It will also be clear that those skilled in the art will conceive of departures from the precise specification of my processes and reagents, 115 as above set forth, employing however the underlying elements and actions called for by the broader of the appended claims. It will also be clear that certain elements may be omitted without departing from the novel 120 advantages gained by the other elements and the proportions may be changed.

I claim:

1. A developer for dyed fabrics including the reaction products of the mixture of beta naphthol, caustic soda, acetic acid, chloroform, zinc acetate, aqua ammonia, alpha naphthylamin, phenol, sodium chlorid, a mineral acid and water substantially as described.
2. The method of producing a developer for treating previously dyed fabric which consists in heating to fusion a mixture of acetic acid, chloroform, zinc acetate, ammonia, beta naphthol, alpha naphthylamin, phenol, caustic soda and water, adding sodium chlorid and a mineral acid, and then reducing the whole to a finely divided state substantially as described.
3. A developer for dyed fabrics compris-

ing the reaction products of the mixture of the following:

|                              |    |
|------------------------------|----|
| 80 gr. acetic acid 30%.      | 20 |
| 80 gr. chloroform.           |    |
| 80 gr. zinc acetate.         |    |
| 10 gr. aqua ammonia 26%.     |    |
| 880 gr. cold water.          | 25 |
| 5 lb. beta naphthol.         |    |
| 1 lb. alpha naphthylamin.    |    |
| 3 lb. phenol (crystallized). |    |
| 8 lb. caustic soda.          |    |
| 75½ lb. sodium chlorid.      | 30 |
| 5 lb. a mineral acid.        |    |

In witness whereof, I hereunto subscribe my name this 26th day of January, A. D. 1917.

WILLY WOLFF.